

N. T. BACON.

METHOD AND APPARATUS FOR RETTING FLAX AND OTHER FIBERS.  
APPLICATION FILED APR. 26, 1917.

1,258,083.

Patented Mar. 5, 1918.



# UNITED STATES PATENT OFFICE.

NATHANIEL T. BACON, OF PEACE DALE, RHODE ISLAND.

## METHOD AND APPARATUS FOR RETTING FLAX AND OTHER FIBERS.

1,258,083.

Specification of Letters Patent.

Patented Mar. 5, 1918.

Application filed April 26, 1917. Serial No. 164,629.

To all whom it may concern:

Be it known that I, NATHANIEL T. BACON, a citizen of the United States, residing at Peace Dale, R. I., have invented certain new and useful Improvements in Methods and Apparatus for Retting Flax and other Fibers, of which the following is a clear, full, and exact description.

My invention relates to the retting of flax or other fibers, and it has for its object to produce a better grade of fiber and to simplify the control of the retting process.

The retting of flax and other fibers is accomplished principally by two processes, first, by exposure to dew, and second, by steeping in water; in either case the end sought is accomplished by means of fermentative or putrefactive processes. As is well-known, these processes are much accelerated by the use of appropriate temperatures, the best average temperature being generally in the neighborhood of 32° C. My experiments go to show that somewhat different temperatures are advisable for different kinds of fibers, and that better results are obtained by using different temperatures at different stages of the operation. I have also found that different parts of the same plant require somewhat different treatment, as the root, the main stem and the top do not all ret at the same rate under the same conditions, and that consequently it is advisable to compensate the differences by different temperatures for different parts of the same plant.

In order to obtain the best results, it is occasionally necessary to completely check the operation as can readily be accomplished by raising the temperature at any stage to a point where the bacteria produced in the operation are all killed, and then beginning fermentation over again with fresh bacteria.

The final purification can be accelerated by washing the flax with heated fresh water, which is subsequently used in retting successive charges. In this manner the volume of water requisite for retting is materially reduced, which is of considerable importance where this water has to be purified in order to obtain good results and is economical of heat in all cases. Moreover, as the retting process, under the conditions which I employ, in comparatively rapid, the with-

drawal from the flax of the retting water of high bacterial content and the substitution therefor of fresh water of low bacterial content furnishes means for controlling the retting process near the end of the operation and therefore reduces the danger of over-retting. A uniform product is thus easily obtained.

One form of apparatus adapted for the practice of my new method comprises a group of retting units such as tanks or compartments, which are so connected together that a continuous flow of retting liquor may be maintained through any number of consecutive units arranged in a retting series.

In the drawings wherein I have illustrated such an apparatus in a more or less diagrammatic and schematic way,

Figure 1 is a view of a number of the units and associated parts employed in my process;

Fig. 2 is a plan view of one of the units shown in Fig. 1;

Fig. 3 is a vertical section of a unit showing a modified form of heat controlling means; and

Fig. 4 is a plan diagram of a complete battery of units, the connecting and other pipes not being shown in detail.

While I have shown the tanks which constitute the units of my apparatus as arranged in a row, this is not essential, and I may arrange them according to any grouping which circumstances require. Each of the tanks has side walls 2 and a bottom wall 3, and is provided with an opening 4 at the bottom of one side and an opening 6 at the top of the opposite side. In the opening 4 is fitted a pipe 8 provided with a hand-operated valve 10; the upper opening 6 is provided with a pipe 12 having a hand-operated valve 14. The pipes 8 and 12 are connected by a vertical pipe 16 which, extending upward, connects with a fresh water main 18, and, extending downward, connects at its other end with the waste main 20; this pipe 16 has between its junction with the pipe 12 and the fresh water main 20 a hand-operated valve 22, and also has a similar valve 24 between its juncture with the pipe 8 and the waste main 20. This arrangement is duplicated between each pair of adjacent tanks in the series with such adaptations

as to dimensions, etc., as the relative position of the tanks may require, it being understood that the arrangement shown is merely one embodiment of this part of my invention.

The tanks may be grouped into one or more series, and water sent through each series in either direction desired. I have found it generally preferable to cause a flow 10 in such direction that the movement of the water is from the bottom of each tank upward to the top thereof. To accomplish this, fresh water is introduced into the first tank of each series through the pipes 8 and 15 16 by opening the valves 10 and 22 therein, the adjacent valves 14 and 24 being closed. The water rises in the tank and overflows into the pipe 12 on the opposite side of the tank; the valve 14 therein being open as is 20 also the valve 10 for the succeeding tank, while the valves 22 and 24 in the pipe 16 between the two tanks are closed. The flow continues thus through all the tanks in the particular series. The water overflowing 25 through the pipe 12 of the last tank in the series into the adjacent pipe 16 is permitted to discharge into the waste main 20 by opening the valve 24 in said pipe 16; the adjacent valve 8 having been closed.

30 If flow in the opposite direction is desired, the fresh water is introduced at the top of the tank that is to be the first of the series, through the pipes 16 and 12, as may be readily understood. In such case, of course, the series will run from right to left instead of from left to right as in the previous case.

Each tank may be provided with a perforated plate or screen 25 supported a short distance above the bottom of the tank, and 40 on the screen the roots of the flax plants rest with their stems extending upwardly. The water from the pipe 8 can therefore flow across the bottom of the tank and rise evenly through the whole area of the flax mass.

45 Each tank is provided with means for controlling the temperature of the water flowing therethrough, one form of such means comprising a series of horizontal pipes 26 extending around the inside of each tank adjacent the walls thereof. Each of these pipes is connected by short pipes 28 and 30 extending through the wall of the tank to vertical supply manifolds 32 and 34, which are in turn connected to mains 36 and 38. Each 55 of the short pipes 28 and 30 is provided with a valve 40 or 42 respectively. At the opposite side of the tank, the horizontal pipes 26 are provided with short pipes 44 emptying into a discharge manifold 48 and each fitted 60 with an automatic check valve 46 to prevent return flow from the manifold. One of the mains, as 36, supplies cold water or other cooling medium, and the other main, that is 38, supplies hot water, steam or the like. It 65 is therefore apparent that by the proper

manipulation of the valves 40 and 42 to cause a flow of cooling or heating fluid through a selected pipe 26, the temperature of the water at different levels may be readily controlled. The manifold 48 empties into waste 70 main 20.

In Fig. 2 I have shown a modification of the temperature controlling means, which consists in providing the pipes 26 with perforations 27 and replacing the check valves 75 46 in the pipes 44 with hand-operated valves 47. With this structure I may introduce the regulating fluid, either gas or liquid, directly into the water, the bubbling of gas through the water being a particularly effective 80 means of controlling its temperature. Gas (by which term I mean to include compressed air, steam or other non-liquid fluid) may also be introduced into the water by means of perforated pipes 50 extending across the 85 bottom of the tank and supplied from a gas main 52. The perforated pipes are also utilized to regulate the temperature by drawing off water from different levels in the tanks; this is accomplished by opening the appropriate valve 47 and permitting water to discharge into the discharge manifold 48, this water being replaced by inflowing water from an adjacent tank or the fresh water main. I have found that in this manner the 90 line of temperature demarcation at a given point can be made quite sharp, the temperature gradient due to the slow conduction of heat between the pipes and the center of the tank being avoided.

95 The water overflowing from one tank into the next may have its temperature changed by the introduction of a temperature regulating medium thereinto. In the form illustrated, an extension 54 from each cold water 105 manifold 26 opens into the adjacent pipe 12 and is provided with a valve 56, the cooled overflow water when entering the next tank tends to spread out over the bottom of the tank and establish a sharply defined zone of 110 lowered temperature about the roots of the flax.

115 As pointed out above the retting of flax goes on at a maximum speed at a temperature of about 32° C. and it can be retarded either by raising the retting fluid above this point or by dropping it therebelow. If the water is to move up from the bottom of the tank to the top, it is generally advisable to regulate by heating but if the water is to 120 move in the opposite direction, there are advantages in regulation by cooling.

125 It will, as a rule, be advantageous by the use of the temperature controlling means to cool or heat the water at the point where the retting is to be retarded, and then to restore the water to about 32° C. as it reaches portions of the flax where retting should be accelerated. If it is found that the main stem is being retted too rapidly, it is only 130

necessary to increase the temperature just above the root, and all above this point will ret more slowly when the flow of water is upward. If the bottom is retting too fast, 5 the temperature here is lowered below the point of maximum retting; this may be accomplished as set forth above by chilling the retting liquor as it overflows from the top of the preceding tank, or by means of 10 the temperature regulating element at the bottom of the tank. By the employment of the temperature controlling means above described, to differentiate the temperatures of the portions of the retting water to the action 15 of which different parts of the flax are subjected, and to independently vary these temperatures, the whole retting operation in each tank comes under control and it is possible to produce a local retardation of the 20 retting process to offset differences in the natural retting speed of the different parts of the flax so as to bring out the entire plant in uniformly retted condition, which has not been accomplished hitherto except accidentally. 25

When the system is in operation, there will be a series of tanks, each of which has been put into operation at a later date than the preceding tank of the series, the intervals 30 between the starting of successive tanks depending upon factors not here material. The number of tanks in series will depend on the amount of flax that the retting water can treat without becoming too foul with 35 the products of the retting action to be effectively used. As the flax in the oldest tanks in the series is subjected to the least contaminated water, a great deal of the impurities are gradually removed in these tanks.

40 The fresh water entering the first tank of the series has practically no retting bacteria therein, so that it is to a considerable extent merely a wash water. In its passage through the flax in this tank, it picks up bacteria, but 45 even when it leaves this tank its bacterial content is low. Therefore the action in the second tank is less rapid than in the presence of retting water of a higher bacterial content, such as flows through the later tanks 50 in the series. The retting action is therefore slowed down in the second tank.

As the flow of the water through the tanks is very slow, there will, notwithstanding the low bacterial content of the water in the 55 first tank, be an appreciable retting action therein. This action may be lessened by heating the wash water considerably above 32° C. The control of the latter part of the retting operation is thus facilitated and it 60 may readily be stopped at the exact point desired. The heating of the wash water also aids in the removal by the solution of the gummy matter remaining in the flax; this heated water will ordinarily be recooled before entering the next tank, as by bubbling 65

gases therethrough by means of the perforated pipes.

When the retting action in the first tank of the series is complete, it is cut off from the series, the next succeeding tank being 70 made the first and a new tank being added to the discharge end of the series. The water is drained off from the cut out tank and the retted flax is removed. Fresh flax is put in and the tank is now ready to be again 75 introduced into the series at the discharge end thereof. It will be seen, therefore, that the series of tanks in which retting is taking place progresses around the circuit of the entire group such as shown in Fig. 4, each 80 tank being in turn made the last of the series, that is, the last to receive the retting water, and thereafter by degrees becoming the first of the series. As each tank is taken out of the series, an examination of the flax 85 therein will enable the attendant to estimate the stage reached by the next tank and the interval before the latter is taken out will accordingly be lengthened or shortened.

It may sometimes be advisable to divide 90 a group of tanks into two or more series following each other around the circuit of the group; that is, after a tank has been cut off from the fresh water end of its series, emptied and refilled, it will be connected to 95 the discharge end of the following series.

In order to reduce the evolution of ill-smelling gases, which are ordinarily given off in the later stages of the retting process and which are considered to be caused by 100 the growth in the retting liquor of different kinds of bacteria than those present in the earlier and inoffensive stages of the retting, the temperature of the contents of a tank in which these later developed bacteria have 105 obtained a foothold may be raised to approximately 95° C., thus destroying all the bacteria and completely stopping the fermentation; after which the fermentation, that is the retting, is started again with 110 liquor which has been taken from some other stage of the retting operation and in which the undesirable bacteria have not appreciably developed.

While I have above set forth specific details of a preferred form of my improved apparatus and method, it is to be understood that both are capable of modification within the scope of the appended claims, and that it is not my intention that in the practice of my invention it shall be limited to the use of the exact structure or mode of procedure herein described. 115

What I claim is:—

1. A method of retting flax or the like, 125 which consists in locally checking the retting action.

2. A method of retting flax or the like, which consists in differentiating the temperatures of the portions of the retting me- 130

dium to the action of which different parts of the flax or the like are subjected.

3. A method of retting flax or the like, which consists in independently varying the 5 temperatures of the portions of the retting medium to the action of which different parts of the flax or the like are subjected.

4. A method of retting flax or the like, which consists in differentiating the 10 temperatures of the portions of the retting medium to the action of which different parts of the flax or the like are subjected, and independently varying the temperatures of said 15 different portions to cause the retting of said different parts to proceed simultaneously.

5. An apparatus for the water retting of flax and the like, comprising a tank for the 20 retting water and the flax, and means for causing a difference in temperature between portions of the retting water at different 25 levels in said tank.

6. An apparatus for the water retting of flax and the like, comprising a plurality of 25 interconnected tanks for the retting water, and independent means for controlling the 30 temperatures of the water at different levels in each tank.

7. A method of controlling fermentation which consists in completely stopping the 30 fermenting action and starting the same anew.

8. A method of controlling fermentation, which consists in destroying the fermentative 35 bacteria in the fermentative medium and adding thereto a new supply of fermentative bacteria.

9. A method of retting flax or the like, which consists in subjecting the flax to the 40 influence of media which are alternately promotive of and opposed to retting action.

10. A method of retting flax or the like, which consists in subjecting the flax to the 45 action of a retting medium, completely stopping said action, and starting said action anew.

11. A method of retting flax and the like, which consists in subjecting flax to a retting 50 medium of high bacterial content until the retting action is nearly complete, then subjecting the flax to a retting medium of low bacterial content and finally washing the completely retted flax in clear water.

12. A method of retting flax or the like, which consists in treating different lots of 55 flax with retting water of high bacterial content, withdrawing the retting water from one lot, washing said lot in fresh water, withdrawing the retting water from a sec-

ond lot, and treating said second lot to the action of the wash water from the first lot. 60

13. A method of retting flax or the like, which consists in subjecting the flax to a retting water of normal temperature until the retting action is nearly complete, and then subjecting the flax to water of relatively 65 high temperature to dissolve the gummy matter remaining in the flax and to make the last part of the retting operation relatively slow.

14. An apparatus for the water retting of 70 flax or the like, comprising a series of tanks for the retting water and the flax in which the flax remains throughout the operation, and means comprising connections between each pair of adjacent tanks for maintaining 75 a constant flow of water through said tanks.

15. An apparatus for the water retting of flax or the like, comprising a group of tanks for the retting water and the flax in which the flax remains throughout the operation, and means comprising connections between said tanks for maintaining a flow of water through successive tanks, said connections being arranged so as to permit the arrangement of said tanks into separate series. 80 85

16. A method of retting flax or the like in a series of tanks, which consists in subjecting the flax in one tank to a retting water of normal temperature until the retting operation is nearly complete, subjecting the flax to water of relatively high temperature to dissolve the gummy matter remaining in the flax and to make the last part of the retting operation relatively slow, and then cooling the water to the proper 90 temperature for the succeeding tank by bubbling appropriate gases therethrough.

17. A method of regulating the water retting of flax, which consists in selectively subjecting portions of the retting water to 100 the direct action of a gas.

18. A method of regulating the water retting of flax, which consists in selectively subjecting portions of the retting water to the direct action of a gaseous temperature 105 regulating medium.

19. A method of regulating the water retting of flax, which consists in bubbling gas through selected portions of the retting water. 110

Signed at Santa Barbara, Calif., this 20th day of April, 1917.

NATHANIEL T. BACON.

Witnesses:

R. J. HAZARD,  
MARY B. B. HAZARD.